

# UNITED STATES PATENT OFFICE.

THOMAS J. MAYALL, OF READING, MASSACHUSETTS.

## COMPOUND SUBSTANCE FOR ELECTRIC INSULATORS.

SPECIFICATION forming part of Letters Patent No. 243,782, dated July 5, 1881.

Application filed May 7, 1881. (No specimens.)

*To all whom it may concern:*

Be it known that I, THOMAS J. MAYALL, of Reading, in the county of Middlesex and State of Massachusetts, have invented a new and 5 useful Improvement in a Compound Substance from which Electric Insulators in any form may be made, of which the following is a specification.

My invention relates to the compound of 10 materials of which the insulating substance is made and the manner of combining and treating them to produce it.

The object of this invention is to produce a substance which shall be, as nearly as possible, 15 a perfect non-conductor of electricity, which can be molded or cut, sawed, turned, or carved in any desired form, and which will combine strength and durability, and at a moderate cost; and it consists in making a compound mass 20 consisting of rubber, graphite, and sulphide or sulphuret of antimony in proportions, by weight, as follows: to one pound of rubber one-quarter of a pound to two pounds of graphite and one-half a pound to two pounds of 25 sulphide or sulphuret of antimony. These are thoroughly commingled and blended together into a plastic mass, and cured by heat to the consistency of "hard rubber," so called.

Insulating articles may be molded from the 30 compound mass before it is cured, and then cured; or masses of the compound may be cured, and desired insulating articles cut from it and worked into the shape required, and finished and polished as metals and hard wood 35 are finished and polished.

To cure this compound I heat it in an oven, as hard rubber is cured, or in any practicable manner, for about one hour at 232° Fahrenheit, one-half hour at about 235°, one-half hour

at 240°, one-half hour at 245°, one-half hour at 40 about 250°, one-half hour at about 255°, one-half hour at about 260°, one-half hour at about 265°, one-half hour at about 270°, one-half hour at about 275°, one-half hour at about 280°, one-half hour at about 285°, one-half hour at about 290°, one-half hour at about 295°, and one hour at about 300°—in all about eight hours, when it will be found to be sufficiently hard and with the most perfect insulating qualities.

From this substance I make all the parts of 50 electrical machines and apparatus and instruments which it is necessary or desirable to have made of non-electric conducting or insulating substance, and also boxes and cases to contain such when in use, and tanks for chemicals used. It may be used instead of glass 55 for insulators to sustain telegraph-wires on the poles.

Iron or other metals and substances may be coated to a considerable thickness with the 60 plastic compound, and then heated, as before described, to cure the compound.

I claim as new and of my invention—

1. The above-described compound substance for electric insulators, consisting of rubber, 65 graphite, and sulphide or sulphuret of antimony blended together and cured by heating, substantially as described.

2. As a new article of manufacture, insulators and insulating articles made of or from a 70 compound of rubber, graphite, and sulphide or sulphuret of antimony, substantially as described.

THOS. J. MAYALL.

Witnesses:

CHS. HOUGHTON,  
H. KENNEY, Jr.